

# United States Patent

Stefan et al.

[15] 3,650,851

[45] Mar. 21, 1972

[54] **GALLIUM CONTAINING COLD-ROLLED TRANSFORMER LAMINATIONS AND SHEETS WITH A CUBIC STRUCTURE**

[72] Inventors: Mihaly Stefan; Fulop Balazs; Zoltan Hegedus; Laszlo Tapolcai, all of Budapest, Hungary

[73] Assignee: Csepeli Femmu

[22] Filed: July 7, 1969

[21] Appl. No.: 839,683

[30] **Foreign Application Priority Data**

July 17, 1968 Hungary.....SE-1433

[52] **U.S. Cl.**.....148/31.55, 75/123 R, 75/123 K, 75/125, 148/111

[51] **Int. Cl.**.....H01f 1/16, C22c 39/46, C22c 39/00

[58] **Field of Search**.....148/31.55, 110, 111, 112, 113, 75/123 R, 123 K, 125

[56]

**References Cited**

**UNITED STATES PATENTS**

|           |         |                   |           |
|-----------|---------|-------------------|-----------|
| 3,008,857 | 11/1961 | Mobius.....       | 148/111   |
| 3,239,332 | 3/1966  | Goss .....        | 75/125    |
| 3,337,373 | 8/1967  | Foster et al..... | 148/31.55 |

**FOREIGN PATENTS OR APPLICATIONS**

|           |         |                    |         |
|-----------|---------|--------------------|---------|
| 651,295   | 10/1962 | Canada.....        | 148/110 |
| 713,034   | 8/1954  | Great Britain..... | 148/111 |
| 1,372,975 | 8/1964  | France.....        | 148/110 |

*Primary Examiner*—L. Dewayne Rutledge

*Assistant Examiner*—G. K. White

*Attorney*—Young & Thompson

[57]

**ABSTRACT**

Cold-rolled transformer laminations with a cubic structure, containing a maximum of 4 percent by weight of silicon alloyed with 0.0001–0.20 percent by weight of gallium, 0–0.5 percent by weight of nickel and 0–0.5 percent by weight of copper.

4 Claims, No Drawings

**GALLIUM CONTAINING COLD-ROLLED  
TRANSFORMER LAMINATIONS AND SHEETS WITH A  
CUBIC STRUCTURE**

The invention concerns cold-rolled transformer laminations and sheets with a cubic texture. The invention further concerns a process for the manufacture thereof.

It is known that the appearance in 1935 of transformer laminations with a so-called Goss texture resulted in great advances in transformer construction. Such laminations can be magnetized most easily in the direction of rolling and their magnetic properties are particularly good in the direction of rolling. Thus e.g., the power loss  $V_{10}$  of a lamination of thickness 0.35 mm. is not more than 0.48 w./kg., while its induction  $B_{25}$  in a magnetic field of 25 AW/cm. equals 18,900 G. In the transverse direction, i.e., at right angles to the direction of rolling, however, the magnetic properties are less advantageous: the power loss  $V_{10}$  is about 1.37 w./kg., whilst  $B_{25}$  is only about 12,200 G. Due to the poor magnetic properties in the transverse direction, only those transformers can be manufactured from transformer laminations with a Goss texture, wherein the direction of the magnetic lines of force coincide with the direction of rolling of the lamination (e.g., sectional lamination cores).

It is further known that both in cold-rolled, as well as in hot-rolled transformer laminations and sheets with isotropic magnetic properties, the magnetic properties are only slightly different in the rolling and transverse directions but the optimum magnetic properties which may be achieved with these laminations, are greatly inferior to the corresponding properties of laminations with a Goss texture: the power loss  $V_{10}$  is 0.8-1.5 w./kg., and the induction with a field intensity of 25 AW/cm. has a value of 14,500 G.

For exacting electrotechnical applications the magnetic properties of the isotropic laminations and sheets are not adequate; such requirements can only be met by transformer laminations with a cubic structure, which can most readily be magnetized in two directions, namely in the direction of rolling and in the transverse direction in the plane of the sheet.

Transformer laminations with a cubic texture have various advantages, the following being the most important:

- a. the magnetic properties are extremely advantageous: the power loss  $V_{10}$  is 0.4-0.6 w./kg. in the longitudinal, as well as in the transverse direction, the initial permeability ( $\mu_s$ ) is 1,500-5,000 G/Oe, and the maximum permeability ( $\mu_s$ ) reaches 25,000-50,000 G/Oe;
- b. the favorable magnetic properties are approximately equal in the longitudinal and transverse directions, which makes possible the manufacture of the various E-, U- and M-cores by simple methods;
- c. by means of the cold-rolled transformer laminations with a cubic texture, magnetic properties can be achieved, which are equivalent to those of 45 percent iron-nickel alloys (e.g., Permalloy B), whereby, however, the induction is far superior to the values obtainable with the iron-nickel alloys.

For a manufacture of laminations sheets with a cubic texture, the most important, known processes are given in the following:

- a. an alloy containing 2.0-4.0 percent of Si or, instead of part of the Si-component, aluminum, and into which also 0.05-0.3 percent of manganese and a small amount of nickel can be alloyed, is hot-rolled to a thickness of about 3.0 mm., then cold-rolled with three to five intermediate annealings to 0.04-0.20 mm., and finally thermally treated for a longer period (for at least 24 hours) at 1,200°-1,300° C. in a dry hydrogen atmosphere with a dew point below -50° C.;
- b. as is known, the cubic texture can be improved by arranging nickel alloys or nickel-containing ceramic materials near the surface of the lamination during the last thermal treatment;
- c. the formation of the cubic texture can also be improved by carrying out the last two intermediate annealings between 1,100° and 1,300° C.;

- d. the cubic texture can advantageously be influenced while respecting certain requirements in that a small amount of hydrogen sulphide is added to the gas amount of hydrogen sulphide is added to the gas atmosphere in the course of the final thermal treatment;
- e. as is known, it is possible to manufacture transformer laminations with a cubic structure starting from a steel ingot crystallized directionally by suitable methods, after an advantageously chosen hot-rolling, subsequent thermal treatment and cold-rolling performed with intermediate treatment, if during the final thermal treatment a dry hydrogen atmosphere or a vacuum is applied;
- f. for manufacturing lamination with a cubic texture, a finished, Goss-textured lamination can be rolled further in two steps with intermediate annealing, after which the final thermal treatment described under (a) is to be used;
- g. finally it is known to produce silicon-iron laminations with a cubic texture by means of the original direction of rolling with respect to 45° or 90° rollers in the plane of the sheet.

All these known processes have the common disadvantage that they require a very strict observation of the manufacturing technique. Even a small change in the rolling system (number of deformations, degree of the individual deformations) or in the intermediate annealing, or minor changes in the content of impurities of the alloy, influence the formation of the cubic texture considerably. The fact that with the same particle orientation, different magnetic properties can occur is a further disadvantage of the known processes. Precisely for these reasons it is very difficult to manufacture transformer laminations with a cubic structure on an industrial scale.

It is the object of the invention to avoid the grave disadvantages of the known methods and to provide a process, by means of which transformer laminations can be mass-produced in a simple manner and at low cost.

The invention is based on the following findings:

1. If a certain amount of gallium is added to the steel containing at most 4 percent by weight of Si, the magnetic properties of the iron-silicon alloys vary most advantageously, the cubic texture formation is considerably increased, the material becoming, however, less sensitive to variations in the rolling and thermal treatment techniques.

Of the numerous advantageous effects of alloying with gallium, the following may be mentioned:

- a. the temperature of the primary recrystallization is varied;
- b. the number of particles in the cubic texture position, formed during the primary recrystallization is increased so that the secondary recrystallization can consequently be carried out at lower temperatures, whereby the particle size becomes more uniform. All this has an advantageous effect on the magnetic properties, and the quantity of cubic texture-oriented particles reaches 80-90 percent;
- c. due to the presence of the gallium traces dissolved in the metal, the crystal surface and crystal boundary energies are considerably varied during the final thermal treatment, i.e., these values are influenced favorably relative to the cubic texture formation;
- d. due to the change in duration of the final thermal treatment and, if desired, the use of the magnetic field during cooling, the adjustment of the ratios of the initial and maximum permeabilities of the laminations with a cubic structure is made possible within wide limits.

2. The action of the gallium alloy can be improved by adding certain quantities of one or more further metals (e.g., nickel or copper).

Both findings are surprising since hitherto it has been assumed that for the manufacture of transformer laminations with a cubic structure it is preferable to keep the content of impurities and alloying materials of the iron-silicon alloys as low as possible and the presence of all alloying constituents, except manganese, aluminum and silicon, was considered to be decidedly disadvantageous.

3. In the case of gallium or of an alloy of gallium with further metals, the best way of avoiding sticking together of the windings and the oxidation or soiling of the lamination surface during the final thermal treatment is to interpose or insert a wire or strip, consisting of an iron alloy containing 0.5-6 percent by weight of aluminum.

The cold-rolled transformer laminations with a cubic texture according to the invention contain a maximum of 4 percent by weight of silicon, alloyed with 0.0001-0.20 percent by weight, preferably 0.04-0.06 percent by weight of gallium, 0.05 percent by weight, preferably 0.2-0.4 percent by weight of nickel, 0-0.5 percent by weight, preferably 0.2-0.3 percent by weight of copper.

The invention further concerns a method for the manufacture of such cold-rolled transformer laminations and sheets with a cubic texture, by micro-alloying the iron-silicon base material by successive thermal shaping, descaling, cold-rolling, intermediate annealing, final rolling and final thermal treatment of the ingot obtained. According to the invention one proceeds in such a manner that the micro-alloying of the steel containing at most 4 percent by weight of silicon is effected with 0.0001-0.20 percent by weight, preferably 0.04-0.06 percent by weight of gallium, 0-0.5 percent by weight, preferably 0.2-0.4 percent by weight of nickel and 0-0.5 percent by weight, preferably 0.2-0.3 percent by weight of copper and, if desired, prior to the final thermal treatment, during the winding up of laminations a wire or strip consisting of an iron alloy containing 0.5-6.0 percent by weight of aluminum is used as a separating means between the lamination windings or core parts.

Of the principal advantages of the process according to the invention, the following may be mentioned hereinbelow:

- a. as against the known processes for the manufacture of laminations with a cubic structure, the process according to the invention is more simple and may be carried out with higher technological tolerances;
- b. the initial and maximum permeabilities, coercive force and induction, as well as the power loss of the lamination with a cubic texture can be considerably improved;
- c. about 80-90 percent of the particles are in the cubic texture position in the end product;
- d. laminations as well as finished cores and parts can be subjected to the final thermal treatment;
- e. the process can be carried out by using known apparatus for the manufacture of transformer laminations with a Goss texture.

Several examples for carrying out the process according to the invention are given in the following.

#### Example 1

An iron-silicon alloy with a nominal content of 3.2 percent of silicon, 0.05 percent of gallium and 0.35 percent of nickel with a very small content of impurities, is produced in an induction vacuum furnace from a pure iron charge of good quality, from metallic silicon with a silicon content exceeding 98.5 percent and with an aluminum content of less than 0.5 percent, as well as from metallic nickel. The impurities of the alloy do not exceed the following values: 0.05 percent of carbon, 0.015 percent of sulphur, 0.03 percent of chromium, 0.03 percent of molybdenum, 0.93 percent of vanadium, 0.03 percent of tungsten, 0.01 percent of titanium and 0.005 percent of oxygen.

The ingot is hot-rolled to a thickness of 3 mm. at a starting temperature of 1,100°-1,150° C. The temperature of the lamination is kept above 900° C. before the last pass.

The scale is removed from the hot-rolled lamination by means of a pickling agent containing sulphuric acid and the lamination is then annealed for 2 hours at 800° C. in a humid hydrogen atmosphere with a dew point of +20 C. The lamination is then cold-rolled in several passes to a thickness of 0.80 mm. and, after degreasing, thermally treated for 2 hours at a temperature of 850° C. in a hydrogen atmosphere with a dew point of -30° C. The lamination is then cold-rolled in several passes to a thickness of 0.30 mm. and, after degreasing, ther-

mally treated for 2 hours at a temperature of 1,000° C. in a vacuum of 10<sup>-3</sup> Torr.

The lamination, the surface of which is metallically pure, is cold-rolled with polished rollers in several passes to a thickness of 0.10 mm. A ribbed strip made of steel containing 1.5 percent of aluminum having a clean surface, is inserted between the windings of the degreased lamination. The thus prepared lamination coil is subjected to a thermal treatment in a vacuum furnace in a vacuum of 10<sup>-3</sup> Torr in such a way that during heating the material is kept hot for 2 hours between 550° and 700° C.; the temperature is then raised to 1,100° C. and kept for 20 hours at this value. After completing the thermal treatment, the charge together with the furnace is cooled to 500° C. 85 percent of the particles of the lamination thus produced are in the cubic texture position; the initial permeability  $\mu_5$  of the lamination is 4,200 G/Oe and the maximum permeability 45,000 G/Oe.

#### Example 2

A lamination cold-rolled according to Example 1 to 3 mm. and produced from a steel ingot, the composition of which corresponds to that of Example 1, is descaled in a pickling agent containing sulphuric acid and then subjected for 2 hours to thermal treatment at 800° C. in a humid hydrogen atmosphere with a dew point of 20° C. The lamination is then cold-rolled to 1.0 mm. in several passes and, after degreasing, thermally treated for 2 hours at a temperature of 850° C. in a hydrogen atmosphere with a dew point of -30° C. The lamination is then cold-rolled in several passes to a thickness of 0.45 mm. and then—after degreasing—subjected for 2 hours to thermal treatment at a temperature of 1,000° C. in a vacuum of 10<sup>-3</sup> Torr.

The lamination, the surface of which is metallically pure, is finally cold-rolled with polished rollers in several passes to a thickness of 0.20 mm. Thereafter one proceeds as in Example 1.

The initial permeability  $\mu_5$  of the lamination thus produced is 4,100 G/Oe and the maximum permeability 37,000 G/Oe.

#### Example 3

One proceeds as described in Example 1 but the silicon content of the alloy is adjusted to 2.6 percent by weight, the nickel content to 0.3 percent by weight and the gallium content to 0.05 percent by weight.

The initial permeability  $\mu_5$  of the lamination thus obtained is 4,000 G/Oe and the maximum permeability 38,000 G/Oe.

#### Example 4

One proceeds as described in Example 1 but the final thermal treatment is carried out for 5 hours.

The initial permeability  $\mu_5$  of the lamination thus obtained is 3,300 G/Oe and the maximum permeability 24,500 G/Oe.

#### Example 5

One proceeds as described in Example 1 but the final thermal treatment is carried out in a dry hydrogen atmosphere (dew point below -50° C.) at 1,200° C. in such a way that this temperature is maintained for 20 hours. In this manner a lamination is obtained, the initial permeability of which is 3,700 G/Oe and the maximum permeability 37,000 G/Oe.

#### Example 6

One proceeds as described in Example 1 except that prior to the final thermal treatment the desired core sheets are cut out from the lamination, and the thermal treatment is carried out in such a way that during cooling and on reaching 700° C. the core sheets are exposed to the action of the magnetic field of a field intensity of 10-20 Oe. The initial permeability  $\mu_5$  of the maximum permeability 63,000 G/Oe.

We claim:

1. Cold-rolled transformer lamination with a cubic structure, consisting essentially of up to 4 percent by weight of silicon, 0.001-0.20 percent by weight of gallium, 0-0.5 percent by weight of nickel and 0-0.5 percent by weight of copper, balance essentially iron.

2. Cold-rolled transformer lamination as claimed in claim 1, in which said gallium is 0.04-0.06 percent by weight, said nickel is 0.2-0.4 percent by weight and said copper is 0.2-0.3 percent by weight.

3. Cold-rolled transformer lamination as claimed in claim 1, in which said silicon is about 3.2 percent by weight, said gallium is about 0.05 percent by weight and said nickel is about 0.35 percent by weight.

4. Cold-rolled transformer lamination as claimed in claim 1, 5 in which said silicon is about 2.6 percent by weight, said nickel is about 0.3 percent by weight and said gallium is about 0.05 percent by weight.

\* \* \* \* \*

10

15

20

25

30

35

40

45

50

55

60

65

70

75